

1

2,881,107

**AUSTEMPERED, COLD-FINISHED STEELS**

Elliot S. Nachtman, Park Forest, Ill., assignor to LaSalle Steel Co., Hammond, Ind., a corporation of Delaware

No Drawing. Application October 22, 1956  
Serial No. 617,268

8 Claims. (Cl. 148—12)

This invention relates to a new and improved metallurgical process applicable to the cold finishing of steels and it relates to a process of the type described capable of producing steels having new and improved characteristics and new and improved combinations of properties.

This invention is related to the processes described in the copending applications Ser. No. 518,411, Ser. No. 518,412, Ser. No. 518,413 and Ser. No. 518,414, filed June 27, 1955 now Patents No. 2,767,837, No. 2,767,835, No. 2,767,836, and No. 2,767,838, respectively.

It is an object of this invention to produce and to provide a method for producing new and improved steels having new and different physical and mechanical properties and combinations thereof.

More specifically, it is an object of this invention to provide a method, adapted for use in the cold finishing of steels, which may be employed to improve certain physical and mechanical properties in the steel, which may be employed to produce steels having new and different combinations of properties thereby to provide new and improved steel products which provide for greater uniformity in properties and characteristics of the steels of corresponding chemistry from heat to heat by comparison with the normal hot rolled steels which are cold finished, which may be employed to expand the range of physical and mechanical properties capable of being developed in the steels thereby to open up new and different areas of use, and it is a related object to produce steels having new and improved characteristics and new and improved physical and mechanical properties.

In the aforementioned copending applications, description is made of a metallurgical process which may be employed in the cold finishing of steel to improve physical and mechanical properties of the steel. The metallurgical process defined is based upon an elevated temperature reduction step wherein, for example, the steel is advanced through a die to take a reduction in cross-sectional area while the steel is at a temperature within the range of 200° F. to the lower critical temperature for the steel composition or while the steel is at a temperature within the range of 200° F. to 1100—1200° F. Depending upon the temperature of the steel reduced in the elevated temperature reduction step, various physical and mechanical properties of the steel can be changed, and in many instances materially improved, by comparison with the same steels given an equivalent reduction but while the steel is at room temperature. Thus, by controlling the temperature of the steel in the elevated temperature reduction step, by controlling the chemistry of the steel and by controlling the amount of reduction, it has become possible to produce new and improved steel products having new and improved physical and mechanical properties and different combinations thereof.

In my copending application filed concurrently herewith and entitled "Cold Finished Steels and Method for the Manufacture of Same," Ser. No. 617,264, description is made of a modification in the elevated temperature reduction concept wherein, prior to the elevated tem-

2

perature reduction step, the steel is heated to austenitizing temperature followed by quenching to produce a phase change in the steel wherein the steel is characterized by the presence of bainite and martensite, alone or in combination. In another copending application filed concurrently herewith and entitled "Metallurgical Process for Cold Finishing Steel," Ser. No. 617,266, description is made of another modification which embodies the elevated temperature reduction concept wherein the steel, prior to taking the elevated temperature reduction step, is austenitized by heating above its transformation range and quenched to effect the described phase change followed by tempering the quenched steel. In each of these processes, utilization continues to be made of the characteristics in the steel whereby improvements are secured in physical and mechanical properties by reduction in cross-section when worked at elevated temperatures.

The process forming the subject matter of this invention embodies a still further modification in the elevated temperature reduction concept. In accordance with the practice of this invention, the hot rolled steels are processed through a combination of steps which includes the step of austempering the hot rolled steel and then advancing the steel through a die to effect the desired reduction in cross-sectional area while the steel is at a temperature within the range of 200° F. to the lower critical temperature for the steel composition and preferably while the steel is at a temperature within the range of 450° F. to the lower critical temperature for the steel composition. The combination of steps which includes austempering the steel prior to taking the elevated temperature reduction step results in the formation of steels characterized by improvements in the strength properties of the steels and in the hardness of the steels over similar steels given an equivalent reduction at elevated temperature without previous austempering and over steels given an equivalent reduction in cross-sectional area by cold drawing following austempering.

Included amongst the physical and mechanical properties which are influenced by the concepts described are the strength properties of the steel, such as tensile strength, impact strength, yield strength, flexural strength and the like and such other properties as elasticity, elongation, hardness, surface roughness, machinability, proportional limits and the like. The most significant improvements developed in steels processed in the manner described are the strength properties of the steel and its hardness.

The characteristics described are capable of development with hot rolled steels of the type which are generally cold finished, as by the processes of drawing or extrusion. Steels which exhibit improvements when processed in accordance with the practice of this invention are similar to those which are beneficially affected by the elevated temperature reduction steps described in the aforementioned copending applications. Such steels are characterized by the ability to strain harden or harden by some mode of precipitation or other re-arrangement when worked at an elevated temperature within the range of 200° F. to the lower critical temperature for the steel composition. Representative are the non-austenitic steels having a pearlitic structure in a matrix of free ferrite. While steels containing carbon over a fairly wide range can be employed, as defined in the aforementioned copending applications, best results are secured in the practice of this invention in the processing of steels having a carbon content greater than 0.040 percent.

In the process embodying the features of this invention, the temperature of the steel in the elevated temperature reduction step, the chemistry of the steel and the amount of reduction influence the level of improvements which are secured and the combination of characteristics and

properties that are capable of being developed in the steel product. By proper selection of temperature, chemistry and reduction, it is possible to produce steels having new and different physical and mechanical properties and it becomes possible selectively to produce steels having low stress characteristics, as will hereinafter be pointed out.

Treatment of the steels after the elevated temperature reduction step, as by slow cooling in air or by quenching rapidly to cool the steel, has little effect upon the characteristics and properties developed in the steel other than the fact that rapid cooling tends to produce steels having a preponderance of compressive stresses to provide steels characterized by negative warpage values, especially when the elevated temperature reduction step is taken while the steel is at a temperature of above 700° F.

As used herein, the term "elevated temperature reduction (ETD)" is meant to include the step of processing the steel wherein the steel is advanced through a die, such as a draw die, extrusion die or roller die, to effect reduction in cross-sectional area while the steel is at a temperature within the range of 200° F. to the lower critical temperature for the steel composition and preferably while the steel is at a temperature within the range of 450° F. to 1100-1200° F. While not equivalent from the standpoint of the process, many of the characteristics described are capable of being developed by other methods for working the steel to effect reduction in cross-sectional area while the steel is at the desired elevated temperature. For example, many of the described improvements are secured in steels which have been austempered and then reduced in cross-section by rolling while the steel is at a temperature within the range of 200° F. to the lower critical temperature for the steel composition.

The term "austempering" is intended to have the same meaning as is normally applied to the term in the art. Briefly described, austempering is intended to relate to a special heat treating process wherein the steel heated to a temperature above the transformation range or to a temperature within the range of 1500-1600° F. is quenched in a medium having a rate of heat abstraction sufficiently high to prevent the formation of high temperature transformation products and maintaining the steel at a temperature below that of pearlitic formation and above that of martensite formation ( $M_s$ ), until transformation is complete.

The following will illustrate the practice of this invention with 4140 steel, which may be considered as representative of the steels capable of being improved by the concepts described and which has the following

The hot-rolled steel bars, as received, were descaled by pickling in sulphuric acid and limed to prevent rusting. The pickled and limed bar stock was then heated in a suitable heat treating furnace to a temperature of 1550° F. for about 45 minutes. The austenitized steel was then quenched in a salt bath maintained at a temperature of 640° F. which is slightly above the martensite formation range and which causes heat abstraction at a rate to avoid passage of the steel through the pearlitic range.

10 The steel was held in the bath for a time sufficient to reduce the temperature uniformly through the steel to about 640° F. (about 16 minutes), and then the steel was cooled to room temperature as by means of a quench or by air cooling.

15 It will be understood that the process of austempering to produce a steel having a low temperature transformation structure is well known to those skilled in the art such that detailed description of the various modifications with respect to the time and temperature relationship need not be set forth in greater detail.

20 The austempered steel was reheated to a desired temperature for advancement through the die to effect reduction in cross-sectional area. A suitable drawing compound was applied to the surfaces of the austempered steel and the steel was advanced through a draw die to effect reduction in cross-sectional area.

25 The properties developed in the steel will hereinafter be set forth in the following table. The advantage of quenching, as compared to air cooling, after drawing appears to reside principally in the reduction of residual stress characteristics, especially when use is made of a temperature in the upper range, preferably above 700° F., in the elevated temperature reduction step. As a result, it will be expedient, in the data hereinafter presented, merely to set forth the values secured as a result of air cooling following drawing. It will be understood that similar properties, other than lower residual stress characteristics, will be secured by quenching the steel in oil or water after the elevated temperature reduction step.

30 In the data hereinafter set forth, comparisons will also be made with the value secured with the same steel, as received in hot rolled condition, with the same steel cold drawn to effect equivalent reduction in cross-sectional area, with the same steel drawn at elevated temperature without previous heat treatment to austemper the steel, with the same steel as quenched to room temperature and austempered by quenching from 640° F. In the drawing operations, 4140 steel of  $1\frac{1}{16}$  inch round 35 was drawn to take a reduction of 19.9 percent.

Table I

[4140 steel austempered at 1550° F. and quenched to 640° F. Drawn to take a 19.9 percent reduction—air cooled after drawing.]

| Temp. of Draw, °F.            | Pull, Lbs. | Tensile Strength, p.s.i. | Yield Strength, p.s.i. | Elongation, Percent | Red. of area, Percent | Hardness, DPH |     |     |
|-------------------------------|------------|--------------------------|------------------------|---------------------|-----------------------|---------------|-----|-----|
|                               |            |                          |                        |                     |                       | S             | MR  | C   |
| Hot Roll                      |            | 140,000                  | 105,750                | 15.0                | 42.8                  | 310           | 307 | 301 |
| Cold Drawn                    | 18,320     | 160,000                  | 153,000                | 9.0                 | 48.9                  | 324           | 330 | 324 |
| ETD <sup>1</sup>              | 15,171     | 195,000                  | 191,250                | 10.0                | 36.7                  | 389           | 402 | 402 |
| As quenched (O) <sup>2</sup>  |            | 292,000                  | 246,000                | 12.9                | 44.1                  | 600           | 429 | 468 |
| Austemper Quench From 640° F. |            | 178,000                  | 136,250                | 13.6                | 57.4                  | 378           | 307 | 307 |
| 690                           | 27,480     | 217,000                  | 217,000                | 9.3                 | 45.7                  | 425           | 462 | 479 |
| 810                           | 20,610     | 184,000                  | 180,250                | 15.0                | 52.6                  | 391           | 333 | 328 |
| 1,000                         | 11,220     | 141,000                  | 120,000                | 21.4                | 58.5                  | 310           | 307 | 302 |

<sup>1</sup> Data at approximate peak of ETD curve.

<sup>2</sup> Conventionally quenched in oil to room temperature.

ladle analysis in which the major ingredients other than iron are set forth:

|            |        |
|------------|--------|
| Carbon     | .33    |
| Manganese  | .88    |
| Phosphorus | .018   |
| Sulphur    | .020   |
| Silicon    | .26    |
| Chromium   | .86    |
| Molybdenum | .18 75 |

70 From the results given, it will be apparent that improvements are secured in the strength properties of the steel and in hardness when the steels are processed in accordance with the practice of this invention by comparison with elevated temperature reduction alone and over cold drawn steels, with or without previously austempering.

It will be evident that by the combination of steps

comprising austempering and elevated temperature reduction improvement can be introduced into steel products thereby to provide a new and improved steel having improved characteristics and different combinations of characteristics by comparison with steels of the type heretofore capable of being produced by various processing techniques.

It will be understood that the invention may be practiced on steel rods, wires, tubing and the like, as well as on bar stock and that changes may be made with respect to the techniques of heating and cooling the steel and in their method of handling through the various process steps without departing from the spirit of the invention, especially as defined in the following claims.

I claim:

1. The metallurgical process of treating steel of the non-austenitic type having a pearlitic structure in a matrix of free ferrite comprising the combination of steps of austempering the steel and then advancing the austempered steel through a die to effect a reduction in cross-sectional area while the steel is at a temperature within the range of 200° F. to the lower critical temperature for the steel composition.

2. The metallurgical process of treating steel which strain hardens and which hardens by some mode of precipitation when worked at a temperature within the range of 200° F. to the lower critical temperature for the steel composition comprising the combination of steps of austempering the steel and advancing the steel through a die to effect a reduction in cross-sectional area by a drawing operation while the steel is at a temperature within the range of 200° F. to the lower critical temperature for the steel composition.

3. The metallurgical process of treating steel which strain hardens and which hardens by some mode of precipitation when worked at a temperature within the range of 200° F. to the lower critical temperature for the steel composition comprising the combination of steps of austempering the steel and advancing the steel through an extrusion die to effect a reduction in cross-sectional area by an extrusion operation while the steel is at a temperature within the range of 200° F. to the lower critical temperature for the steel composition.

4. The metallurgical process of treating steel which strain hardens and which hardens by some mode of precipitation when worked at a temperature within the range of 200° F. to the lower critical temperature for the steel composition comprising the combination of steps of

austempering the steel and rolling the steel to effect a reduction in cross-sectional area by a rolling operation while the steel is at a temperature within the range of 200° F. to the lower critical temperature for the steel composition.

5. The metallurgical process of treating steel which strain hardens and which hardens by some mode of precipitation when worked at a temperature within the range of 200° F. to the lower critical temperature for the steel composition comprising the combination of steps of austempering the steel and advancing the steel through a die to effect a reduction in cross-sectional area while the steel is at a temperature within the range of 200° F. to the lower critical temperature for the steel composition, and air cooling the steel after the elevated temperature reduction step.

6. The metallurgical process of treating steel which strain hardens and which hardens by some mode of precipitation when worked at a temperature within the range of 200° F. to the lower critical temperature for the steel composition comprising the combination of steps of austempering the steel and advancing the steel through a die to effect a reduction in cross-sectional area while the steel is at a temperature within the range of 200° F. to the lower critical temperature for the steel composition, and quenching the steel rapidly to cool the steel after the elevated temperature reduction step.

7. The metallurgical process of treating steel which strain hardens and which hardens by some mode of precipitation when worked at a temperature within the range of 450° F. to the lower critical temperature for the steel composition comprising the combination of steps of austempering the steel and advancing the steel through a die to effect a reduction in cross-sectional area while the steel is at a temperature within the range of 450° F. to the lower critical temperature for the steel composition.

8. A steel having new and improved physical and mechanical properties produced by the method of claim 5

#### References Cited in the file of this patent

#### UNITED STATES PATENTS

2,435,511 Rice ----- Feb. 3, 1948

#### OTHER REFERENCES

Metals Handbook, 1948 ed., pages 286 and 629.

Pomp: The Manufacture and Properties of Steel Wire, copyright 1941, English translation, 1954, pages 205-233 and 92-93.